

# UNITED STATES PATENT OFFICE.

GADIENT ENGI, OF BASEL, SWITZERLAND, ASSIGNOR TO SOCIETY OF CHEMICAL INDUSTRY IN BASLE, OF BASEL, SWITZERLAND.

## PROCESS FOR PRODUCING FAST TINTS.

1,245,694.

Specification of Letters Patent.

Patented Nov. 6, 1917.

No Drawing.

Application filed November 4, 1915. Serial No. 59,647.

To all whom it may concern:

Be it known that I, GADIENT ENGI, a citizen of the Swiss Republic, and resident of Basel, Switzerland, have invented a new 5 Process for Producing Fast Tints, of which the following is a full, clear, and exact specification.

In the application for United States Letters Patent Ser. No. 43413, filed August 3, 1915, and in the two applications for United States Letters Patent of Berthold Wuth and Carl Jagerspacher, Ser. Nos. 54503 and 54504, filed October 7, 1915, is described the production of new copper 10 compounds of orthooxyazodyestuffs yielding by their dyeing in an acid bath on animal fibers tints which are fast to light, washing and alkali; however, the fastness of the thus produced dyeings of fulling and potting is 15 not perfect. I have now made the technically valuable observation that those of the copper compounds of orthooxyazodyestuffs able to be produced according to the aforesaid applications for Letters Patent, which 20 contain, besides the copper saturated hydroxyl group proceeding from the orthoxydiazocompound, still one or several groups able to be combined with chromium, as for instance a carboxyl group in the diazo- 25 compound, or a hydroxyl group and a carboxyl group in the component combined with the diazo-compound, can be transformed into chromium lake on the fiber. Hereby the shades of the acid dyeings are 30 not changed or only little changed, but simultaneously the fastness to fulling and potting are increased in such a manner that they 35 satisfy the highest demands. The conversion of the said copper compounds of ortho- 40 oxyazodyestuffs into the new chromium lakes on the fiber can be obtained by dyeing the same on chromium mordanted wool or by dyeing the same from a bath containing simultaneously soluble salts containing 45 chromium, as for instance chromates or chromium salts or by treating the said dyeings subsequently with soluble salts containing chromium, as for instance chromates or chromium salts.

As the copper compounds of the ortho- 50 oxyazodyestuffs yield nearly without exception considerably more vivid tints than those hitherto obtained by treating the acid dyeings of orthooxyazodyestuffs subsequently with chromium compounds or by dyeing 55 with the said orthooxyazodyestuffs according to the metachromium process and as the acid dyeings of the copper compounds have, as already pointed out, their shades not changed or not essentially changed by their 60 conversion into chromium lake, the new process permits producing much more vivid tints than those obtainable heretofore with orthooxyazodyestuffs dyeing on mordants, the fastness of the dyeings obtained by the 65 new process being without exception at least equal and in part still better than those of the latter dyestuffs. The new process resolves the important problem to furnish the hitherto obtained increasing of fastness by 70 subsequent treatment with chromium compounds, without any change of the shades of the acid dyeings, whereby obtaining of pre-determined final shades is facilitated.

The copper compounds of the aforesaid 75 oxyazodyestuffs are furthermore also suitable for the production of fast tints on vegetable fibers, by dyeing or printing these latter on cotton according to the processes usually employed for dyestuffs dyeing on mordants, whereby the said copper compounds 80 are transformed on the fiber into chromium lakes showing excellent fastness to washing and to light. That could not have been foreseen, as all hitherto prepared orthooxyazo- 85 dyestuffs dyeing or mordants were not suitable for cotton dyeing.

As parent materials for the new process can be employed the copper compound or orthooxyazodyestuffs obtainable according 90 to three above mentioned applications for U. S. Letters Patent, which contain, besides the copper saturated hydroxyl group originating from the oxydiazocompound, still a rest able to be combined with chromium, as 95 for instance a carboxyl group in the diazo-compound or a hydroxyl and a carboxyl group in the component coupled to the

diazocompound. The introduction of such a group able to be combined with chromium can for instance be effected by starting from aminooxycarboxylic acids of the benzene and naphthalene series, as for instance,



30      further from other aminooxycarboxylic acids, as for instance,



45      and combining the same after diazotization with any component to orthooxymono-, dis- or polyazodyestuffs. Or any orthooxydiazocompounds, as for instance, orthooxydiazophenol-sulfonic acid, nitroorthooxydiazophenolsulfonic acid, etc., is combined with salicylic acid, the various oxynaphthoic acids, paracetaminic acid, the pyrazolones derived from aminosalicylic acid as for instance



etc. The orthooxyazodyestuffs thus obtained are transformed in the known manner into the corresponding copper compounds or

these latter can also be obtained by effecting the said combination in presence of copper derivatives (copper salts, copper oxid, copper hydroxid, etc.).

The employ of the obtained copper compounds for the production of fast tints by their transformation into chromium lakes on the fiber is illustrated by the following examples:

(a) ANIMAL FIBERS. 75

*Example 1.*

*Dyeing of the copper compounds on previously applied mordant.*

Wool is mordanted as usually with 3% potassium chromate and 2.5% potassium bitartrate. The so mordanted wool is dyed in a bath containing 3 to 5% acetic acid of 40% and 1 to 3% dyestuff (copper compound), the goods being introduced into the bath at 50-60° C., the bath slowly heated to boiling and the boiling maintained for 1 to 1½ hours. 80

*Example 2.* 90

*Dyeing of the copper compounds with addition of chromates or chromium oxid salts to the bath.*

The dyeing bath for 100 kg. wool is prepared with 15 to 20 kg. crystallized sodium sulfate, 3 to 5 per cent. acetic acid of 40%, the necessary quantity of dyestuff (copper compound) and of potassium chromate (the half of the dyestuff weight) and the material to be dyed is introduced into the bath at a temperature of 50 to 60° C. The bath is slowly heated to boiling and maintained in ebullition for ¾ to 1 hour and exhausted by a further boiling for ¼ hour after an addition of 1 to 2 kg. formic acid of 90%. Instead of potassium chromate can be employed salts of chromium oxid. 95

*Example 3.* 110

*Subsequent treatment of the copper compounds with chromium compounds.*

The dyeing bath is prepared with 1 to 3% dyestuff (copper compound), 10 to 15% crystallized sodium sulfate and 3 to 5% acetic acid of 40%. The well moistened wool is introduced into the bath at a temperature of 50 to 60° C. and the bath is heated in the course of half an hour to boiling. After a boiling for ¾ hour, ½ to 1% sulfuric acid is added and the bath is boiled for a further quarter of an hour. After an addition of some cold water to the bath, potassium chromate (½ quantity of the dyestuff employed) is added to the same and the wool chromated for ½ to ¾ hour. 115

Instead of starting from the achieved cop-

- per compounds of the orthooxyazodyestuffs, the copper compounds can be produced directly on the unmordanted animal fiber and the obtained dyeings of the copper compounds be treated subsequently with chromium, or the copper compounds can be produced directly on chromium mordanted fibers. Finally the orthooxydiazodyestuffs or their sodium salt, which contain, besides the hydroxylgroup proceeding from the orthoxydiaz compound, still a group able to combine with chromium, can be dyed by adding simultaneously copper salts and chromates to the bath, whereby the shades of the copper compounds of the said dyestuffs are obtained with the excellent fastness of the chromium lakes.

*Example 4.*

- 20 *Production of the copper compounds on previously mordanted goods.*

The wool is mordanted as usually with 3% potassium chromate and 2.5% potassium bitartrate.

25 The dye bath is prepared with 1 to 3% dyestuff (sodium salt), 2 to 3% copper sulfate and 3 to 5% acetic acid of 40%. The wool is introduced in the bath at a temperature of 50 to 60° and the bath heated slowly to boiling and boiled for 1 to 1½ hours.

*Example 5.*

- 35 The dyeing bath is prepared with 1 to 3% dyestuff (sodium salt), 2 to 3% copper sulfate, 10% crystallized sodium sulfate, 3 to 5% acetic acid of 40% and a quantity of potassium chromate equal to the half weight of the employed dyestuff, the goods being introduced in the bath at a temperature of 50 to 60° C. and the bath being heated to boiling and boiled for 1 to 1½ hours.

40 To obtain a better exhaustion of the bath 1 to 1.5% formic acid of 90% can be added to the same, after a further boiling for ¼ of an hour to 1 hour.

*Example 6.*

- 50 The dyeing bath is prepared with 1 to 3% dyestuff (sodium salt), 2 to 3% copper sulfate, 10% crystallized sodium sulfate and 3 to 5% acetic acid of 40%. The material is introduced in this bath at a temperature of 55 50 to 60° C. and the bath slowly heated to boiling and boiled for ¾ of an hour to 1 hour. Hereafter, in order to obtain a better exhaustion of the bath, 1 to 1.5% formic acid of 90% are added and the bath is further boiled for ¼ of an hour.

55 After dyeing the bath is allowed to cool slightly, a quantity of potassium chromate

equal to the half weight of the dyestuff employed is added thereto and the material is chromated in the boiling bath for ½ an hour 65 to ¾ of an hour.

Instead of being utilized for dyeing, the various dyestuffs can also be employed for the printing of animal fibers according to the usual process by adding acid or chromium salts to the printing color. 70

*Example 7.*

10 to 20 gr. dyestuff (copper compound) 75 are dissolved in 270 to 230 ccm. water and mixed with 700 gr. British gum thickening and 20 to 50 gr. tartaric acid of 50% or 10 to 20 gr. dyestuff (copper compound) are dissolved in 280-240 ccm. water and mixed with 650 gr. British-gum thickening, 10 gr. 80 tartaric acid of 50% and 50 to 80 gr. chromium acetate or the corresponding quantity of chromium fluorid.

The paste is printed on chlorinated wool goods, and this latter is steamed in a 85 moistened state, for 1 hour, washed and terminated as usually.

*(b) VEGETABLE FIBERS.*

*Example 8.*

*For cotton dyeing.*—Chromium mordanted cotton is dyed in a bath containing 1 to 3% dyestuff (copper compound) and 2½ to 5% acetic acid of 40%, the goods being introduced in the cold bath and the latter afterward slowly heated to boiling and maintained in ebullition for ½ an hour. 95

Instead of starting from the achieved copper compound, this latter can be produced on chromium mordanted cotton by dyeing the goods in a boiling bath containing 1 to 3% dyestuff, 2 to 3% copper sulfate and 2 to 5% acetic acid of 40%. 100

*Example 9.*

*For cotton printing.*—10 to 30 parts dyestuff (copper compound) are dissolved in 250 ccm. hot water containing eventually 1 to 2 ccm. soda lye of 30% and the resulting solution is mixed with 640 to 570 gr. of a neutral starch-British gum-thickening, 50 ccm. acetic acid of 40% and 50 to 100 ccm. chromium acetate. The paste is printed on 115 cotton, and the goods steamed for 1 hour, washed and terminated as usually in the printing of chromium dyestuffs.

The dyestuffs can also be employed in the usual discharge printing processes. 120

With the specified dyestuffs the most various tints of excellent fastness to light and washing can be produced on vegetable fibers.

In the following tabular exhibit are indi-

cated various dyestuffs applicable with the new process and the comparative dyeings of their sodium salts and of their copper compounds:

| Dyestuff derived from— |                                            | Dyeing of the sodium salt. |                         | Dyeing of the copper compound. |                         |
|------------------------|--------------------------------------------|----------------------------|-------------------------|--------------------------------|-------------------------|
| Diazo compound of—     | And the following component—               | Acid.                      | Subsequently chromated. | Acid.                          | Subsequently chromated. |
|                        | 1:8-Amidonaphthol-2:4-disulfonic acid..... | Red violet.....            | Dull green blue.        | Violetish blue....             | Blue.                   |
|                        | 1:8-Amidonaphthol-2:4-disulfonic acid..... | Red violet.....            | Black violet.....       | Pure greenish blue.            | Greenish blue.          |
| "                      | 1:8-Amidonaphthol-3:6-disulfonic acid..... | Red violet.....            | Black violet.....       | Greenish blue...               | Greenish blue.          |
| "                      | 1:8-Dioxynaphthalene-3:6-disulfonic acid   | Red violet.....            | Dark blue.....          | Violet.....                    | Violet.                 |
| "                      | 1:4-Naphtholsulfonic acid.....             | Pure bluish red.....       | Bordeaux.....           | Bordeaux.....                  | Bordeaux.               |
| "                      | 1:5-Naphtholsulfonic acid.....             | Bluish red.....            | Blackish bordeaux.      | Bluish bordeaux                | Pure bluish bordeaux.   |
| "                      | 2:6-Naphtholsulfonic acid.....             | Yellowish red...           | Bordeaux.....           | Bluish red.....                | Bluish red.             |
| "                      | 2:8-Amidonaphthol-6-sulfonic acid.....     | Violet brown....           | Black brown....         | Yellowish black brown.         | Yellowish black brown.  |
| "                      | 1:5-Amidonaphthol-7-sulfonic acid.....     | Dull red violet..          | Violetish brown.        | Red violet.....                | Red violet.             |
| "                      | 2-Naphthol-3:6-disulfonic acid.....        | Bluish red.....            | Bluish bordeaux.        | Strong bluish red.             | Strong bluish red.      |
|                        | 1-Naphthol-3:8-disulfonic acid.....        | Pure red.....              | Yellowish bordeaux.     | Pure blue bordeaux.            | Bordeaux.               |
| "                      | 1-Naphthol-3:6-disulfonic acid.....        | Pure bluish red.           | Violet bordeaux.        | Bordeaux.....                  | Bordeaux.               |
| "                      | 2:5-Amidonaphthol-7-sulfonic acid.....     | Yellowish red...           | Yellowish bordeaux.     | Pure bordeaux..                | Pure bordeaux.          |
| "                      | Benzoyl-2:5-amidonaphthol-7-sulfonic acid. | Yellowish red...           | Bordeaux.....           | Bordeaux.....                  | Bordeaux.               |
| "                      | Phenyl-2:5-amidonaphthol-7-sulfonic acid.  | Yellowish red...           | Yellowish bordeaux.     | Bluish bordeaux.               | Bluish bordeaux.        |
| "                      | m-Amidophenol.....                         | Yellowish brown            | Red brown.....          | Black brown....                | Black brown.            |
| "                      | Salicylic acid.....                        | Brown olive....            | Bronce brown...         | Brown olive....                | Brown olive.            |
| "                      | o-Cresotinic acid.....                     | Brown olive....            | Red olive.....          | Brown olive....                | Brown olive.            |
| "                      | Resorcinol.....                            | Yellowish brown            | Red brown.....          | Brown.....                     | Brown.                  |
| "                      | $\beta$ -Oxynaphthoic acid.....            | Reddish brown.             | Violet brown....        | Brown.....                     | Brown.                  |
| "                      | 3-Oxy-1-thionaphthene.....                 | Red.....                   | Red brown....           | Bordeaux.....                  | Bordeaux.               |
| "                      | Dicetohydroindene.....                     | Red orange.....            | Red orange.....         | Yellow brown...                | Yellow brown.           |

| Dyestuff derived from—                                                              |                                                                                                                               | Dyeing of the sodium salt. |                         | Dyeing of the copper compound. |                         |
|-------------------------------------------------------------------------------------|-------------------------------------------------------------------------------------------------------------------------------|----------------------------|-------------------------|--------------------------------|-------------------------|
| Diazo compound of—                                                                  | And the following component—                                                                                                  | Acid.                      | Subsequently chromated. | Acid.                          | Subsequently chromated. |
|    | o-Carboxylated benzoylacetic acid.....<br>   | Brown.....                 | Destroyed.....          | Blue violet.....               | Blue violet.            |
|    | $\beta$ -Naphthol.....                                                                                                        | Yellow red.....            | Yellowish bordeaux.     | Red.....                       | Red.                    |
| "                                                                                   | 1:5-Naphtholsulfonic acid.....                                                                                                | Blue red.....              | Violet brown...         | Blue red.....                  | Blue bordeaux.          |
| "                                                                                   | 2:6-Naphtholsulfonic acid.....                                                                                                | Yellow red.....            | Red.....                | Red.....                       | Red.                    |
| "                                                                                   | $\alpha$ -Naphthylamin.....                                                                                                   | Yellow brown...            | Brown.....              | Red brown.....                 | Brown.                  |
| "                                                                                   | 1:5-Amidonaphthol.....                                                                                                        | Violet brown...            | Black brown...          | Black brown...                 | Black brown.            |
| "                                                                                   | $\beta$ -Oxynaphthoic acid.....                                                                                               | Bluish bordeaux.           | Dull violet.....        | Bordeaux.....                  | Bordeaux.               |
| "                                                                                   | $\alpha$ -Oxynaphthoic acid.....                                                                                              | Red brown.....             | Violet brown...         | Brown.....                     | Brown.                  |
| "                                                                                   | 1:4-Naphtholsulfonic acid.....                                                                                                | Blue red.....              | Violet.....             | Bluish red.....                | Bluish red.             |
| "                                                                                   | 1:8:5-Amidonaphtholsulfonic acid.....                                                                                         | Red blue.....              | Blue black.....         | Red blue.....                  | Red blue.               |
| "                                                                                   | 1:8-Amidonaphthol-2:4-disulfonic acid...                                                                                      | Red violet.....            | Dull blue.....          | Pure blue.....                 | Pure blue.              |
|  | 1-Phenyl-3-methyl-5-pyrazolone.....                                                                                           | Yellow orange...           | Red orange.....         | Reddish yellow.                | Reddish yellow.         |
| "                                                                                   | Diamidodiphenylamindisulfonic acid...                                                                                         | Orange brown...            | Red brown.....          | Brown.....                     | Brown.                  |
| "                                                                                   | Acetacetic-anilid.....                                                                                                        | Lemon yellow...            | Green yellow...         | Green yellow...                | Green yellow.           |
| "                                                                                   | 3-Oxy-1-thionaphthene.....                                                                                                    | Red.....                   | Brown red.....          | Red violet.....                | Red violet.             |
| "                                                                                   | Dicetohydroinden.....                                                                                                         | Orange.....                | Yellow red.....         | Red brown.....                 | Brown.                  |
| "                                                                                   | Perinylphthindion...                                                                                                          | Orange.....                | Yellow red.....         | Brown.....                     | Yellow brown.           |
| "                                                                                   | o-Carboxylated benzoylacetic acid.....<br> | Brown.....                 | Destroyed.....          | Pure blue.....                 | Pure blue.              |

| Dyestuff derived from— |                                          | Dyeing of the sodium salt. |                         | Dyeing of the copper compound. |                         |
|------------------------|------------------------------------------|----------------------------|-------------------------|--------------------------------|-------------------------|
| Diazo compound of—     | And the following component—             | Acid.                      | Subsequently chromated. | Acid.                          | Subsequently chromated. |
|                        | 1:8-Amidonaphthol-2:4-disulfonic acid... | Blue violet.....           | Greenish blue...        | Greenish blue...               | Greenish blue.          |
| "                      | 1:8-Amidonaphthol-3:6-disulfonic acid... | Red violet.....            | Greenish blue...        | Greenish blue...               | Greenish blue.          |
|                        | 1:5-Naphtholsulfonic acid.....           | Yellow bordeaux            | Blue violet.....        | Blue bordeaux...               | Blue bordeaux.          |
| "                      | 2:3:6-Naphtholdisulfonic acid.....       | Yellow bordeaux            | Blue violet.....        | Bordeaux.....                  | Bordeaux.               |
| "                      | 1:4-Naphtholsulfonic acid.....           | Yellow bordeaux            | Blue violet.....        | Bordeaux.....                  | Bordeaux.               |
| "                      | 2:6-Naphtholsulfonic acid.....           | Red.....                   | Red violet.....         | Bordeaux.....                  | Bordeaux.               |
| "                      | 2:5-Amidonaphthol-7-sulfonic acid.....   | Yellow red.....            | Violet.....             | Violet brown....               | Violet brown.           |
| "                      | 2:8-Amidonaphthol-6-sulfonic acid.....   | Violet brown...            | Black violet....        | Black brown....                | Black brown.            |
| "                      | 1:8-Dioxynaphthalene-3:6-disulfonic acid | Violet.....                | Green blue.....         | Blue violet.....               | Blue violet.            |
| "                      | Phenylmethylpyrazolensulfonic acid.....  | Yellow orange...           | Yellow red.....         | Brown orange...                | Brown orange.           |
| "                      | Resorcinol.....                          | Yellow red.....            | Red brown.....          | Yellow brown...                | Brown.                  |
| "                      | 1:8-Amidonaphthol-4-sulfonic acid.....   | Blue violet.....           | Red brown.....          | Green blue.....                | Green blue.             |
| "                      | 1:4:3-Naphtholdisulfonic acid.....       | Bordeaux.....              | Blue violet.....        | Violet.....                    | Violet.                 |
| "                      | 1:3:8-Naphtholdisulfonic acid.....       | Bordeaux.....              | Blue violet.....        | Red violet....                 | Bordeaux.               |
|                        | 1:8-Amidonaphthol-3:6-disulfonic acid... | Red violet.....            | Bluish green...         | Blue.....                      | Blue.                   |
| "                      | 1:8-Amidonaphthol-2:4-disulfonic acid... | Red violet.....            | Bluish green...         | Blue.....                      | Blue.                   |
|                        | Salicylic acid.....                      | Yellow.....                | Red orange....          | Yellow.....                    | Reddish yellow.         |
| "                      | $\beta$ -Oxynaphthoic acid.....          | Yellowish bordeaux.        | Violet.....             | Bluish bordeaux                | Bluish bordeaux.        |
|                        | $\beta$ -Oxynaphthoic acid.....          | Violet black....           | Violet.....             | Bluish bordeaux                | Bluish bordeaux.        |

| Dyestuff derived from—                                                              |                                                                                     | Dyeing of the sodium salt. |                         | Dyeing of the copper compound. |                         |
|-------------------------------------------------------------------------------------|-------------------------------------------------------------------------------------|----------------------------|-------------------------|--------------------------------|-------------------------|
| Diazo compound of—                                                                  | And the following component—                                                        | Acid.                      | Subsequently chromated. | Acid.                          | Subsequently chromated. |
|    |    | Red brown.....             | Red.....                | Red.....                       | Red.....                |
|    | "                                                                                   | Yellow red.....            | Orange.....             | Yellow orange...               | Yellow orange.          |
|    | "                                                                                   | Red yellow.....            | Red orange.....         | Orange.....                    | Orange.                 |
|   |   | Red orange.....            | Blue red.....           | Blue red.....                  | Blue red.               |
|  |  | Dull violet.....           | Blue green.....         | Pure blue violet.              | Pure blue violet.       |
|  | "                                                                                   | Blue red.....              | Dull violet.....        | Bordeaux.....                  | Bordeaux.               |

| Disazo dyestuff derived from— |                                                    |                                        | Dyeing of the sodium salt. |                         | Dyeing of the copper compound. |                         |
|-------------------------------|----------------------------------------------------|----------------------------------------|----------------------------|-------------------------|--------------------------------|-------------------------|
| The diazo compound of—        | The following to be further diazo-tized component— | And the final component—               | Acid.                      | Subsequently chromated. | Acid.                          | Subsequently chromated. |
|                               | Acid of Cleve....                                  | 2:5-Amidonaphthol-7-sulfonic acid.     | Red blue.....              | Green blue.....         | Blue.....                      | Green blue.             |
| "                             | Acid of Cleve....                                  | 2:6-Naphtholsulfonic acid.             | Red blue.....              | Blue black.....         | Blue.....                      | Blue.                   |
| "                             | Acid of Cleve....                                  | 1:8-Amidonaphthol-3:6-disulfonic acid. | Green blue.....            | Blue green.....         | Green blue.....                | Green blue.             |
| "                             | Acid of Cleve....                                  | 2-Naphthol-3:6-disulfonic acid.        | Blue.....                  | Green blue.....         | Green blue.....                | Green blue.             |

What I claim is:

1. The described process for producing fast tints on animal and vegetable goods, which consists in forming the dye in the presence of the goods by combining a soluble salt containing chromium with a copper compound of orthooxyazodyestuff, which contains besides the copper saturated hydroxyl group proceeding from the orthooxydiazocompound, at least one group capable of being chromated.

15 2. The described process for producing fast tints on animal and vegetable goods, consisting in first dyeing the goods in a bath formed by a solution of a copper compound of orthooxyazodyestuff containing besides the copper saturated hydroxyl group proceeding from the orthooxydiazocompound, at least one group capable of being chromated, and treating afterward the thus obtained dyeings with a solution of a salt containing chromium.

20 3. The described process for producing fast tints on animal and vegetable goods,

consisting in dyeing the goods in a bath 25 formed by a solution of a copper compound of orthooxyazodyestuff containing besides the copper saturated hydroxyl group proceeding from the orthooxydiazocompound, at least one group capable of being chromated, and of a salt containing chromium.

30 4. The described process for producing fast tints on animal and vegetable goods consisting in dyeing the goods with a solution of a copper salt and of an orthooxyazodyestuff containing besides the hydroxyl group proceeding from the orthooxydiazocompound at least one group capable of being chromated and treating the thus obtained dyeings afterward with a solution of a salt 35 containing chromium.

In witness whereof I have hereunto signed my name this 6th day of October 1915, in the presence of two subscribing witnesses.

DR. GADIENT ENGI.

Witnesses:

ARNOLD ZUBER,  
AMAND RITTER.